

## 1

3,181,945

### HIGH STRENGTH STEEL

Arthur R. Elsea, Columbus, Ohio, assignor, by mesne assignments, to The Battelle Development Corporation, Columbus, Ohio, a corporation of Delaware  
 No Drawing. Filed Oct. 5, 1961, Ser. No. 143,066  
 6 Claims. (Cl. 75—123)

This invention relates to ultrahigh-strength steel compositions, and, more particularly, to alloys exhibiting 0.2 percent offset yield strengths of 290,000 p.s.i., or greater, combined with good ductility.

In the design of solid-propellant rocket motors, one of the most critical problems is to find suitable ultrahigh-strength sheet materials from which fuel containers can be fabricated. It is desirable to use ultrahigh-strength materials for this application so as to reduce the weight of the fuel containers. However, in the past, as the strength level of available engineering materials increased, the ductility decreased, and the sensitivity to notches and other inadvertent stress raisers increased. Furthermore, it is characteristic of all structural materials that they exhibit less ductility in the presence of biaxial or triaxial tensile stresses than they do in the presence of uniaxial tensile stresses. Service loads imposed on solid-propellant fuel containers result in fairly severe biaxial tensile stresses, and any type of stress raisers (such as small flaws from the fabrication process, or possibly nonmetallic inclusions or microcracks in the metallic structure) may lead to catastrophic brittle failures at nominal stresses far below the expected strength of the material as determined by uniaxial load.

It is, therefore, an object of this invention to provide alloys possessing ultrahigh tensile strengths with good ductility. It is a further object of this invention to provide steel alloy materials possessed of ultrahigh strengths together with high fracture strengths in the presence of biaxial and triaxial tensile stress, and in the presence of small flaws. Other objects and advantages of the present invention will be apparent from the following detailed description thereof.

In general, this invention comprises alloy steel compositions containing about 0.45 to about 0.60 carbon, about .40 to about 1.25 manganese, about 1.8 to about 2.25 silicon, about 1.2 to about 1.8 nickel, and about 0.16 to about 0.35 vanadium, balance iron. For some applications, the present alloys may also include boron in amounts ranging from about 0.0003 to about 0.01. A preferred composition comprises about 0.5 carbon, about 1.0 manganese, about 2.0 silicon, about 1.5 nickel, about 0.30 vanadium, and, for some applications, about 0.01 boron, balance iron. (All percentages are weight percentages.)

#### EXAMPLE 1

An alloy was prepared having a nominal composition of 0.50 C, 1.0 Mn, 2.0 Si, 1.5 Ni and 0.3 V, balance Fe. The tensile strength of this alloy was found to be 335,000 p.s.i., and the 0.2 percent offset yield strength was 300,000 p.s.i. The alloy exhibited an elongation of 8 percent in 2 inches and a reduction of area of 29 percent.

#### EXAMPLE 2

An alloy having the composition of the alloy of Example 1 plus .01 percent B was prepared. This alloy had a tensile strength of 325,000 p.s.i. and a 0.2 percent offset yield strength of 290,000 p.s.i. However, the elongation increased to 9 percent and the reduction in area increased to 32 percent as compared with values of 8 percent and 29 percent respectively for the alloy composition of Example 1.

## 2

It will be seen from Examples 1 and 2 above that the addition of a small amount of boron has little effect on the strength of the present alloys, but improves the ductility by a significant amount. This effect has been studied in more detail and is illustrated by the data in Table I which show the effect of additions of .0003 to 0.01 percent boron.

Table I.—Effect of boron on mechanical properties of the Ni—V steel<sup>1</sup>

[Refrigerated —125 F., tempered 600 F.]

| Steel designation        | Boron added, percent | Tensile strength, 1,000 p.s.i. | 0.2 percent yield strength, 1,000 p.s.i. | Elongation in 2 inches, percent | Reduction in area, percent |
|--------------------------|----------------------|--------------------------------|------------------------------------------|---------------------------------|----------------------------|
| AUSTENITIZED AT 1,700 F. |                      |                                |                                          |                                 |                            |
| 31                       | 0                    | 333                            | 300                                      | 8                               | 29                         |
| 31-2                     | 0                    | 323                            | 284                                      | 6½                              | 21                         |
| 49                       | 0.0003               | 337                            | 293                                      | 7½                              | 29                         |
| 50                       | 0.010                | 328                            | 291                                      | 9                               | 32                         |
| AUSTENITIZED AT 1,650 F. |                      |                                |                                          |                                 |                            |
| 31-2                     | 0                    | 326                            | 286                                      | 7                               | 25                         |
| 49                       | 0.0003               | 338                            | 307                                      | 7                               | 27                         |
| 50                       | 0.010                | 323                            | 288                                      | 9                               | 32½                        |
| AUSTENITIZED AT 1,550 F. |                      |                                |                                          |                                 |                            |
| 31                       | 0                    | 327                            | 294                                      | 7                               | 24                         |
| 31-2                     | 0                    | 319                            | 283                                      | 7                               | 25                         |
| 49                       | 0.0003               | 334                            | 301                                      | 8                               | 30                         |
| 50                       | 0.010                | 312                            | 275                                      | 9                               | 35                         |

<sup>1</sup> Results obtained with 0.505-inch-diameter specimens.

The data in Table I above support the conclusion that boron additions, in amounts ranging from 0.0003 to 0.01 percent, improve ductility of the high strength alloys without substantially adversely affecting the strength properties.

#### EXAMPLE 3

An alloy having the following composition was prepared: 0.49 C, 1.01 Mn, 2.12 Si, 1.53 Ni, 0.30 V, balance essentially Fe. Transverse and longitudinal properties of this alloy were determined using specimens that were austenitized at 1700° F., oil quenched, refrigerated to —125° F., and then double tempered at 600° F. for about 1 hour each cycle. Properties (average of two or three specimens) determined were as follows:

*Longitudinal properties.*—Tensile strength, 303,000 p.s.i.; 0.2 percent yield strength, 269,000 p.s.i., 0.02 percent yield strength, 217,000 p.s.i.; elongation, 3 percent and hardness, Rockwell C, 50.5.

*Transverse properties.*—Tensile strength, 319,000 p.s.i.; 0.2 percent yield strength, 281,000 p.s.i.; 0.02 percent yield strength, 236,000 p.s.i.; elongation, 3 percent and hardness, Rockwell C, 53.

As has been previously noted in this disclosure, for certain applications, such as rocket motor casings, it is not enough that a material possess ultrahigh strength with ductility; it must also possess what is commonly designated as "fracture strength." Fracture strength is a measure of a material's ability to withstand stress in the presence of a notch, crack, or similar small flaw. Although there is no standard way of determining fracture strength, there are several methods that are used. All of these methods are characterized by the fact that they are complex and involved. In all of them fracture strength usually decreases with increasing tensile strength or yield strength, for a given material.

Using one of the methods for determining fracture

strength, it has been demonstrated that compositions according to this invention have fracture strengths of 200,000 p.s.i. for yield strengths of 240,000 p.s.i. SAE 4340, one of the least notch-sensitive high strength steels, by the same method of determination, has a fracture strength 5 of 200,000 p.s.i. at a maximum yield strength of 215,000 p.s.i. Thus, the compositions of this invention possess yield strengths 25,000 p.s.i. or more greater than the better prior art high strength steels, and, at the same time, 10 retain fracture strengths equivalent to those of the lower strength steels. This combined high fracture strength-high yield strength is unique to the materials of the present invention.

The alloys of this invention may be used as aluminum-killed alloys. For example, the alloy of Example 3 15 was aluminum killed. Whenever B is used in the present alloys then the alloy must be deoxidized with aluminum. In other instances, the alloys may be deoxidized with silicon.

New and useful ultrahigh-strength steel compositions 20 capable of use as fuel containers for solid-propellant rocket motors, or for tension members in aircraft, or for other high-strength applications have been described. These alloys possess an unusual combination of yield strength, reduction in area, elongation properties, and 25 fracture strength wherefore many other advantages and applications for these alloys will be apparent to those skilled in the art. It is desired to define the invention in the following claims which are intended to be interpreted, as to scope, in view of the description in this 30 specification.

What is claimed is:

1. Ultrahigh-strength steel compositions consisting of

from about 0.45 to about 0.60 percent carbon, about .4 to 1.25 percent manganese, about 2.0 to about 2.2 silicon, about 1.2 to about 1.8 nickel, about 0.16 to about 0.35 vanadium, balance essentially iron.

2. Steel compositions according to claim 1 including, in addition, from about 0.0003 to about 0.10 percent boron.

3. Steel compositions according to claim 1 characterized by a 0.2 percent offset yield strength of at least about 290,000 p.s.i.

4. Steel compositions according to claim 1 further characterized by a fracture strength of at least 200,000 p.s.i., at a 0.2 percent offset yield strength of 240,000 p.s.i.

5. Steel compositions according to claim 2 characterized by a 0.2 percent offset yield strength of at least 300,000 p.s.i.

6. Steel compositions according to claim 2 further characterized by a fracture strength of at least 200,000 p.s.i., at a 0.2 percent offset yield strength of 240,000 p.s.i.

#### References Cited by the Examiner

##### UNITED STATES PATENTS

|           |       |           |       |           |
|-----------|-------|-----------|-------|-----------|
| 1,342,911 | 6/20  | Johnson   | ----- | 75—128.85 |
| 2,861,908 | 11/58 | Mickelson | ----- | 75—123    |

##### FOREIGN PATENTS

|         |      |                |
|---------|------|----------------|
| 782,778 | 9/57 | Great Britain. |
|---------|------|----------------|

DAVID L. RECK, *Primary Examiner.*

RAY K. WINDHAM, *Examiner.*

UNITED STATES PATENT OFFICE  
CERTIFICATE OF CORRECTION

Patent No. 3,181,945

May 4, 196

Arthur R. Elsea

It is hereby certified that error appears in the above numbered patent requiring correction and that the said Letters Patent should read as corrected below.

Column 4, line 6, for "0.10" read -- 0.01 --.

Signed and sealed this 26th day of October 1965.

(SEAL)

Attest:

ERNEST W. SWIDER  
Attesting Officer

EDWARD J. BRENNER  
Commissioner of Patents

**Dedication**

3,181,945.—*Arthur R. Elsea*, Columbus, Ohio. HIGH STRENGTH STEEL.  
Patent dated May 4, 1965. Dedication filed Aug. 2, 1974, by the assignee, *The Battelle Development Corporation*.

Hereby dedicates to the People of the United States the entire remaining term of said patent.

[*Official Gazette December 24, 1974.*]